

# United States Patent [19]

Dorn

[11] 3,905,781

[45] Sept. 16, 1975

[54] **CARBURETOR DETERGENT AND CORROSION INHIBITING MOTOR FUEL COMPOSITIONS**

[75] Inventor: **Peter Dorn**, Lagrangeville, N.Y.

[73] Assignee: **Texaco Inc.**, New York, N.Y.

[22] Filed: **Oct. 30, 1972**

[21] Appl. No.: **301,905**

[52] U.S. Cl. .... **44/71; 44/62; 44/80**

[51] Int. Cl. .... **C10l 1/22**

[58] Field of Search..... **44/62, 71, 80**

[56] **References Cited**

UNITED STATES PATENTS

|           |        |                       |         |
|-----------|--------|-----------------------|---------|
| 3,031,282 | 4/1962 | Andress et al.....    | 44/71   |
| 3,046,102 | 7/1962 | Andress et al.....    | 44/71   |
| 3,502,451 | 3/1970 | Moore et al.....      | 44/80 X |
| 3,672,852 | 6/1972 | Vermillion et al..... | 44/62   |
| 3,676,089 | 7/1972 | Morris et al.....     | 44/62   |

Primary Examiner—Patrick P. Garvin

Assistant Examiner—Andrew H. Metz

Attorney, Agent, or Firm—T. H. Whaley; C. G. Ries; J. J. O'Loughlin

[57] **ABSTRACT**

Motor fuel composition comprising a mixture of hydrocarbons in the gasoline boiling range containing an aliphatic hydrocarbon substituted succinamic acid represented by the formula:



in which R is an aliphatic hydrocarbon radical having from about 12 to 20 carbon atoms, and X and Y alternately represent hydrogen and an aliphatic hydrocarbon radical having from 6 to 16 carbon atoms.

**14 Claims, No Drawings**

## CARBURETOR DETERGENT AND CORROSION INHIBITING MOTOR FUEL COMPOSITIONS

### BACKGROUND OF THE INVENTION

#### 1. Field of the Invention

Modern internal combustion engine design is undergoing important changes to meet new federal standards concerning engine exhaust gas emissions. A major change in engine design recently adopted is the feeding of blowby gases from the crankcase zone of the engine into the intake air supply to the carburetor rather than venting these gases to the atmosphere as in the past. Further changes being adopted involve the recycling of a part of the exhaust to the combustion zone of the engine in order to further reduce objectionable emissions. The recycled exhaust gases contain substantial amounts of deposit-forming substances which promote the formation of deposits in and around the throttle plate area of the carburetor. These deposits restrict the flow of air through the carburetor at idle and at low speeds so that an overrich fuel mixture results. This condition produces rough engine idling and stalling, and serves to increase the undesirable exhaust emissions which the engine design changes are intended to overcome.

Modern gasoline compositions are very highly refined products. Despite this, they contain minor amounts of impurities which can promote corrosion during the period that the fuel is transported and stored, and even in the fuel tank, fuel lines and carburetor of the motor vehicle. An acceptable motor fuel must contain a corrosion inhibitor to inhibit or prevent corrosion.

#### 2. Summary of the Invention

A class of aliphatic hydrocarbon substituted succinamic acid compounds are provided as carburetor detergents and corrosion inhibitors when employed in a liquid hydrocarbon fuel for an internal combustion engine. These compounds, which are characterized by having two relatively long hydrocarbon radicals, including one attached to a nitrogen atom, appear to be unique in their carburetor detergency and corrosion inhibiting properties. Similar compounds having additional hydrophilic groups are susceptible to extraction by the tank water bottoms present in fuel distribution systems making it difficult to maintain an effective concentration of the additive in the fuel composition.

The fuel composition of the invention prevents or mitigates the problems of corrosion and deposits lay down in the carburetor of an internal combustion engine. When a gasoline of the invention is employed in a carburetor which already has a substantial build-up of deposits from prior operations, a rather severe test of the detergency property of a fuel composition, this gasoline is very effective for removing substantial amounts of the pre-formed deposits.

### DESCRIPTION OF THE PREFERRED EMBODIMENTS

The aliphatic hydrocarbon substituted succinamic acid of the invention is represented by the formula:



in which R is an aliphatic hydrocarbon radical having from about 12 to 20 carbon atoms and X and Y alternately represent hydrogen and an aliphatic hydrocarbon radical having from about 6 to 16 carbon atoms.

5 Both aliphatic hydrocarbon radicals can be saturated.

In a preferred embodiment of the invention, X or Y is an alkenyl radical having from about 8 to 14 carbon atoms. R is preferably a saturated aliphatic radical having from 16 to 18 carbon atoms.

10 Methods for preparing the additive of the invention are well known and do not constitute part of this invention.

In a preferred method, an olefinically unsaturated hydrocarbon is reacted with maleic anhydride to produce an alkenyl succinic anhydride. This is then reacted with an aliphatic amine of suitable chain length in 1 to 1 mole proportions at a temperature below about 95°C. to produce an N-alkyl alkenyl-succinamic acid. It will be appreciated that the product can be a mixture of compounds conforming to the alternate versions of the formula given above. It will also be understood that the mixture of compounds can effectively be employed as the additive in the motor fuel of the invention.

15 The following example is typical of the preferred method for preparing the additive:

#### EXAMPLE I

##### N-Tallow Tetrapropenyl Succinamic Acid

30 0.7 equivalent of tallow amine (179 g. of a commercial tallow amine-Armeen-T) and 0.7 equivalent (186 g.) tetrapropenyl succinic anhydride and 365 gm. of xylene are heated with gentle stirring at about 80°C. for approximately 6 hours. The recovery is quantitative, 730 g. of an amber fluid oil.

35 A typical analysis for this product is as follows:

|                    |        |
|--------------------|--------|
| GN                 | 1.6    |
| TAN                | 48     |
| TBN                | 4.8    |
| N <sub>20</sub>    | 1.4900 |
| Sp. Grav. 60/60°F. | 0.8823 |

40

The following compounds are effective as additives in the motor fuel composition of the invention:

N-Tallow Tetrapropenyl Succinamic Acid (mixture of stearyl and oleyl)

45 50 N-Oleyl Tetrapropenyl Succinamic Acid

N-C<sub>15</sub>-C<sub>20</sub> Sec. Alkyl Tetrapropenyl Succinamic Acid (derived from Armeen L-15)

N-C<sub>12</sub> tert. Alkyl Tetrapropenyl Succinamic Acid (derived from Primene 81-R)

55 51 N-C<sub>18</sub>-C<sub>22</sub> tert. Alkyl Tetrapropenyl Succinamic Acid (derived from Primene JM-T)

N-Tallow Dodecyl Succinamic Acid

N-Oleyl Dodecyl Succinamic Acid

N-C<sub>15</sub>-C<sub>20</sub> Sec. Alkyl Dodecyl Succinamic Acid

60 60 N-C<sub>12</sub> tert. Alkyl Dodecyl Succinamic Acid

The prescribed aliphatic hydrocarbon substituted succinamic acid of the invention can be employed in the gasoline fuel composition in a concentration both to provide effective carburetor detergency and corrosion inhibiting properties. In general, the additive is employed in a concentration ranging from about 0.0005 to 0.1 weight percent with a preferred concen-

tration ranging from about 0.002 to 0.075 weight percent.

Any gasoline suitable for a spark-ignited, internal combustion engine can be used in the practice of this invention. In general, the base fuel will consist of a mixture of hydrocarbons in the gasoline boiling range, i.e., boiling from about 75° to 450°F. The hydrocarbon components can consist of paraffinic, naphthenic, aromatic and olefinic hydrocarbons. This gasoline can be obtained naturally or it can be produced by thermal or catalytic cracking and/or reforming of petroleum hydrocarbons. The base fuel will generally have a Research Octane Number above 85 and up to about 102 with the preferred range being from about 90 to 100.

The prescribed aliphatic hydrocarbon substituted succinamic acid additive was tested for effectiveness in the carburetor detergency test. This test is run on a Chevrolet V-8 engine mounted on a test stand using a modified four-barrel carburetor. The two secondary barrels of the carburetor are sealed and the feed to each of the primary barrels arranged so that the detergent additive fuel can run in one barrel and the reference fuel run in the other. The primary carburetor barrels were also modified to contain removable aluminum inserts in the throttle plate area so that the deposits formed on the inserts could be conveniently weighted.

Two procedures were used to determine the effectiveness of additive fuel for removing preformed deposits in the carburetor. In the first procedure, designated I, the engine is run for a period of time, usually 24 to 48 hours, using the base fuel as the feed to both barrels with engine blow-by circulated to the air inlet of the carburetor. The weight of the deposits on both sleeves

fuel and of the additive fuels for removing deposits expressed in percent.

In the second procedure, designated II, the engine is run for a period of time, usually 24 to 48 hours, using the base fuel as the feed to both barrels with engine blow-by circulated to the air inlet of the carburetor. The weight of the deposits on both sleeves is determined and recorded. The engine is then cycled for 24 additional hours with base fuel being fed to one barrel and the additive fuel to the other. During the cycle, engine blow-by is circulated to the air inlet of the carburetor. The inserts are then removed from the carburetor and weighed to determine the difference between the performances of the additive and detergent fuels for removing preformed deposits. After the aluminum inserts have been cleaned, they are replaced in the carburetor and the process repeated with the fuel feeds into the carburetor reversed in order to minimize differences in fuel distribution and carburetor construction. The results obtained in the two runs are averaged and the effectiveness of the base fuel and of the additive fuels for removing deposits expressed in percent.

The base fuel employed in the following examples was a premium grade gasoline having a Research Octane Number of about 100 and containing 3 cc. of tetraethyl lead per gallon. This gasoline consisted of about 25 percent aromatic hydrocarbons, 10 percent olefinic hydrocarbons and 65 percent paraffinic hydrocarbons and boiled in the range from about 90°F. to 380°F.

Fuel compositions of the invention were tested in the Chevrolet Carburetor Detergent Test and the results set forth in Table I below. The percent effectiveness reported is the difference obtained by subtracting the percent effectiveness of the base fuel from the percent effectiveness of the additive fuel.

TABLE I

## CARBURETOR DETERGENCY TEST

| Run | Additive & Conc. (1)                                                                | Test Procedure | Wash Down % (3) | % Effectiveness Δ |
|-----|-------------------------------------------------------------------------------------|----------------|-----------------|-------------------|
|     |                                                                                     |                | Base Fuel       | Additive Fuel     |
| 1.  | N—C <sub>11</sub> —C <sub>11</sub> sec. alkyl tetrapropenyl succinamic acid, 20 PTB | I              | +16             | 59                |
| 2.  | N-tallow tetrapropenyl succinamic acid, 10 PTB (2) (4)                              | II             | +22             | 68                |
| 3.  | N-tallow tetrapropenyl succinamic acid, 7.5 PTB (2)                                 | II             | +6              | 56                |
| 4.  | N-tallow tetrapropenyl succinamic acid, 5 PTB (2)                                   | II             | +26             | 29                |
| 5.  | N-tallow tetrapropenyl succinamic acid, 5 PTB (2) (4)                               | II             | +24             | 49                |

(1) PTB - Additive concentration in pounds per thousand barrels of gasoline.

(2) Additive fuel contained 0.075 vol. percent of polypropylene of about 850 aver. mol. weight and 0.12 vol. percent of petroleum carrier oil.

(3) "+" sign indicates fuel built-up deposits.

(4) Additive also contains an equal weight of vylene.

is determined and recorded. The engine is then cycled for 24 additional hours with base fuel being fed to one barrel and the additive fuel to the other and no blow-by to the carburetor air inlet. The inserts are then removed from the carburetor and weighed to determine the difference between the performances of the additive and non-additive fuels for removing preformed deposits. After the aluminum inserts have been cleaned, they are replaced in the carburetor and the process repeated with the fuel feeds into the carburetor reversed in order to minimize differences in fuel distribution and carburetor construction. The results obtained in the two runs are averaged and the effectiveness of the base

The foregoing data illustrate the surprising effectiveness of the prescribed aliphatic hydrocarbon substituted succinamic acid as a carburetor detergent in a motor fuel composition. In all the runs, the base fuel was ineffective as a carburetor detergent as evidenced by the build-up of deposits. In contrast, the additive fuel removed a substantial amount of the deposits giving results ranging from 55 to 90 percent more effective than the base fuel.

The corrosion inhibiting properties of a gasoline composition of the invention was determined in a corrosion test designated the Colonial Pipeline Rust Test. In this test, a steel specimen, polished with non-

waterproof fine emery paper is immersed in 300 ml of stirred test fuel at 100°F. for 30 min. Then 30 ml distilled water is added and stirred for 3.5 hours. The specimen is visually rated and a rating of <5% rust is considered passing.

The Base Fuel employed in this test is identical to the Base Fuel used in the Examples of Table I above. The results are given in the Table below:

TABLE II

| COLONIAL PIPELINE RUST TEST |                                                                                         |          |
|-----------------------------|-----------------------------------------------------------------------------------------|----------|
| Run                         | Additive & Conc.                                                                        | % Rust   |
| 1.                          | none                                                                                    | 75 to 95 |
| 2.                          | N-tallow tetrapropenyl succinamic acid, 20 PTB                                          | Trace    |
| 3.                          | N-tallow tetrapropenyl succinamic acid, 10 PTB                                          | Trace    |
| 4.                          | N-tallow tetrapropenyl succinamic acid 7.5 PTB*                                         | <5       |
| 5.                          | N-C <sub>11</sub> to C <sub>11</sub> , sec. alkyl tetrapropenyl succinamic acid, 10 PTB | Trace    |

\*Additive also contains an equal amount of xylene.

It is evident from the foregoing data that the novel aliphatic hydrocarbon substituted succinamic acids of the invention are outstandingly effective as rust or corrosion inhibitors in gasoline.

The fuels of the invention may contain any additive conventionally employed in gasoline. Tetraalkyl lead, antiknock additives, dyes, corrosion inhibitors, antioxidants and the like can be beneficially employed without materially affecting the detergent additive of the invention. Gasolines containing from about 0.01 to 0.20 volume percent of a polymer, copolymer or the corresponding hydrogenated polymer or copolymer of a C<sub>2</sub> to C<sub>6</sub> unsaturated hydrocarbon having a molecular weight in the range of 500 to 3,500, preferably from 650 to 2,600, as described in U.S. Pat. No. 3,502,451, which disclosure is incorporated in this application, in combination with the detergent of the present invention are particularly effective multifunctional fuels, compositions containing polypropylene and polyisobutylene of 800 to 1,100 molecular weight at from about 0.025 to 0.1 volume percent being particularly preferred.

I claim:

1. A motor fuel composition comprising a mixture of hydrocarbons in the gasoline boiling range containing from about 0.0005 to 0.1 weight percent of an alkenyl succinamic acid represented by the formula:



in which R is an aliphatic hydrocarbon radical having from about 12 to 20 carbon atoms and X and Y alter-

nately represent hydrogen and an aliphatic hydrocarbon radical having from about 6 to 16 carbon atoms.

2. A motor fuel composition according to claim 1 in which R is an essentially saturated aliphatic hydrocarbon radical.

3. A motor fuel composition according to claim 1 in which R consists predominantly of C<sub>16</sub> and C<sub>18</sub> aliphatic hydrocarbon radicals.

4. A motor fuel composition according to claim 1 in which X or Y is an aliphatic hydrocarbon radical having from about 8 to 14 carbon atoms.

5. A motor fuel composition according to claim 1 in which X or Y is an alkenyl radical.

6. A motor fuel composition according to claim 1 in which X or Y is a tetrapropenyl radical.

7. A motor fuel composition according to claim 1 in which R is an octadecyl radical.

8. A motor fuel composition according to claim 1 in which R is an octadecenyl radical.

9. A motor fuel composition according to claim 1 in which R is a tetradecyl radical.

10. A motor fuel composition according to claim 1 containing from about 0.002 to 0.075 weight percent of said alkenyl succinamic acid.

11. A motor fuel composition according to claim 1 containing from about 0.01 to 0.20 volume percent of (1) a polymer of C<sub>2</sub> to C<sub>6</sub> unsaturated hydrocarbon (2) a copolymer of a C<sub>2</sub> to C<sub>6</sub> unsaturated hydrocarbon, or (3) the corresponding hydrogenated polymer or copolymer, said polymer or copolymer having a molecular weight in the range from about 500 to 3,500.

12. A motor fuel composition according to claim 1 containing from about 0.025 to 0.1 volume percent of polypropylene having a molecular weight ranging from about 800 to 1,100.

13. A motor fuel composition according to claim 1 containing from about 0.025 to 0.1 volume percent of polyisobutylene having a molecular weight ranging from about 800 to 1,100.

14. A method for preventing the build-up of carburetor deposits in an internal combustion gasoline engine which comprises supplying to and burning in said engine a motor fuel composition comprising a mixture of hydrocarbons in the gasoline boiling range containing from about 0.0005 to 0.1 weight percent of an alkenyl succinamic acid represented by the formula:



in which R is an aliphatic hydrocarbon having from about 12 to 20 carbon atoms and X and Y alternately represent hydrogen and an aliphatic hydrocarbon radical having from about 6 to 16 carbon atoms.

\* \* \* \* \*